

May 15, 1934.

F. LIERG

1,958,830

PROCESS OF PRODUCING PHOTOGRAPHS AND CINEMATOGRAPHIC FILMS IN NATURAL COLORS

Filed June 12, 1929

Fig.1



Fig.2



Fig.3



Fig.4



F. Lierg  
INVENTOR

By: Marks & Clark  
A.M.S.

Patented May 15, 1934

1,958,830

# UNITED STATES PATENT OFFICE

1,958,830

## PROCESS OF PRODUCING PHOTOGRAPHS AND CINEMATOGRAPHIC FILMS IN NATU- RAL COLORS

Friedrich Lierg, Dresden, Germany

Application June 12, 1929, Serial No. 370,321  
In Austria August 2, 1928

7 Claims. (Cl. 95—2)

This invention relates to a process of producing photographs and cinematographic films in natural colors in which two or more inseparably superposed layers of silver halid emulsions are utilized, rendered sensitive to the individual spectral sections, which are different among themselves and correspond to the color-synthesis. A photographic material of a number of layers is already known but the results obtained with the same have not been satisfactory in any way, because the hitherto known processes of converting the silver images produced in the individual layers into pigment or color images did not work satisfactorily and positive and cannot be sharply limited to certain layers with a certain degree of positiveness.

It is known that difficulties are encountered in obtaining a correct exposure of the partial color traces which are required for subtractive three color photography and also in obtaining an exact covering thereof after conversion into their corresponding colors. It is not new to endeavor to obviate this drawback and methods of working with a plurality of inseparably superposed layers of silver halid of varying color sensitiveness have already been described (see U. S. Patents 1,516,824 and 1,659,148). It was thereby possible to obtain directly by a single exposure and development partial color silver images superposed in individual layers.

The present invention resides in the fact that the partial color silver images contained in the two layers of emulsion cast on top of each other are converted only by bath treatment into their corresponding colors so that the reactions for producing color are positively confined to the actual layer of emulsion whereby the correctly spectral ground-colors are produced independently of each other. This result is obtained according to the present method by separating a layer, after the production of its corresponding color image, from the other layer by gelatine-hardening in a physical or chemical manner and thereby shutting off further actions during the coloration of the superposed partial color image. In order to produce three color images, a third layer of emulsion is preferably provided on the back of the film where the third partial color image is produced.

In order to produce the color of these two varying ground-colors according to a further very simple mode of carrying out the present process, preferably both partial color images of the double emulsion may be dyed with the same ground-color, for instance, bluish red and after shutting off the lower partial color image the upper partial color image alone is dyed with a suitable dye, for instance, bluish green so that by mixing both dyes the upper image is dyed correctly spectral to its corresponding ground-

color, for instance, pure blue. If an acid dye is used for obtaining a ground-color by redyeing another ground-color while a basic dye has been selected for the uniform preliminary dyeing, it is possible to harden the entire gelatine for shutting off the lower partial color image. The acid dye has a great tendency to chemically combine with the basic dye so that in the case of a slight superficial softening of the hardened gelatine, for instance by the addition of acid to the coloring bath, the entire upper basic color-image, and this alone, attracts the acid dye.

After dyeing the lower partial color image, the gelatine is hardened in such a manner that it repels all dye-solutions either by means of physical agents, i. e. in a known manner by light, or in a chemical manner. If substances are used for this purpose, which oxidize or otherwise tan the gelatine by means of a chemical bath after the dyeing of the lower partial color image, the said substances are preferably added to a layer (for instance, the light-filter layer) arranged between the two emulsions. However, the two partial color images can be separated from each other by hardening the interposed gelatine in a chemical manner by means of the developed silver and without adding any special substances to the gelatine and in the case of emulsions directly cast on top of each other without any intermediate layer. The reaction thus taking place as well as the carrying out of the process to produce by means of emulsions cast on top of each other and without any transfer merely by means of baths a positively selection-correctly dyed three-color photography are explained by the following example.

Four examples of the photographic material necessary for carrying out the process are illustrated in cross section and on an enlarged scale on the accompanying sheet of drawings.

Fig. 1 shows an image base 1 provided with three directly superposed silver halid emulsion layers 2, 3 and 4, which are sensitized for different spectral sections.

Fig. 2 illustrates an image base 1 provided on one side with a single emulsion layer 4 and on the other side with a double layer 2, 3.

Figs. 3 and 4 are views similar to Figs. 1 and 2 respectively, in which however the superposed layers are separated by intermediate layers 5.

The following example, in accordance with Fig. 2 describes one way of carrying out this invention.

As already stated, a film emulsified on both sides is preferably used for taking the picture. It is thus possible by means of any optional division of the image for an exposure to take place from both sides and consequently for the time of exposure to be reduced. Moreover, the dyeing process as well as any desired correction of the obtained colors are considerably simplified. The

most satisfactory arrangement discovered seems to be if the blue-screen negative is produced on the side with the single emulsion, while in the bottom layer of the side with two emulsions the green-screen image and in the upper layer thereof the red-screen image are produced by suitably screening the beam of light and in view of the different sensibilities of the two inseparably cast emulsions. After developing the film and placing the same in an acid bath for interrupting the development, but while the film is not fixed, the blue-screen image on one side is dyed according to any convenient method, for instance by toning with vanadium salt and potassium ferricyanide or over a mordant with a yellow dye, and fixed before the further treatment of the film and protected by a coat of varnish, or the film is treated on one side by merely allowing the same to float.

The double layer side of the film, in which the red and blue part-image is embedded in the still unvaried silver bromid in the form of black silver-images, is treated, for instance according to the last mentioned mode of gelatine-hardening over developed silver, with a mordant-bath which converts the two silver images into mordant images which combine the basic dyes but cannot be reduced by developing agents. While practically all presently known mordant combinations are reduced to metal by reducing agents such as developing agents, it has been found that a suitable mordant resisting development consists according to this process in a silver-copper-sulfocyanid combination, which is produced by bleaching the silver-image in a solution of cupric sulphate and ammonium sulfocyanid to which ammonium oxalate is added. Now if a bluish red dye for instance Rhodamine R index No. 573 is applied this dye attacks the mordant image but not the unchanged silver bromide, because the same does not possess any mordant character. Now the film is exposed to daylight and developed, whereupon the unchanged mordant dye-image is embedded in the black silver. This silver renders possible a picture-like tanning of the gelatine, such as is known for, instance in the case of bromide prints. A solution of chromic acid, potassium bromids and cupric sulphate may constitute a suitable bath for this purpose. This bath bleaches the silver-image and at the same time hardens the gelatine at these places, so that the same repel aqueous dye-solutions after being cleared, washed and dried. If the double layer thus treated is allowed to float on a solution of an acid bluish green dye for instance fast green extra bluish index No. 523 or is bathed therein, a picture-like imbibition of the dye takes place in the known manner at the unhardened places of the gelatine. Under these circumstances, the said imbibition of the dye can only take place in the mordant image on the surface because all other places are shut off by the picture-like tanning and repel the color-solution. Consequently, there is produced in the upper layer a pure blue partial image which consists of the mingling of the original bluish red dyed mordant image with the bluish green imbibition dye image which has only penetrated into the same.

I claim:

1. A method of producing a color photograph comprising inseparably casting on a base superposed silver halid layers of different color-sensitiveness, exposing said layers, developing whereby a non-developed space remains between the partial images, treating the image layers to give

the bottom layer its finish, hardening the non-developed part between said layers, and treating the top layer to give it its finish.

2. A method of producing a color photograph comprising inseparably casting on a base superposed silver halid layers of different color-sensitiveness, exposing said layers, developing whereby a non-developed space remains between the partial images, coloring the latter inversing the images, tanning the latter by a hardening bleaching agent, and treating the upper image layer to obtain an image of different color than the bottom image.

3. A method of producing a color photograph comprising inseparably casting on a base superposed silver halid layers of different color-sensitiveness, exposing said layers, developing whereby a non-developed space remains between the partial images, converting the developed images into special mordant images which are not reducible by a developing agent, dyeing bluish red the mordant images, now developing the remained unfixed silver bromid, tanning the gelatine by a bleaching agent, and redyeing with a bluish green dyestuff the top image to produce a pure blue color image.

4. A method of producing a color photograph comprising casting on a base a silver halid layer, forming on said layer a separating layer of gelatine, inseparably casting on top of said separating layer a second silver halid layer of different color-sensitiveness, producing the images by a single exposure, developing the partial images, treating the image layers to give the bottom layer its finish, hardening said separating layer, and treating the top layer to give it its finish.

5. A method of producing a color photograph comprising casting on a base a silver halid layer, forming on said layer a separating layer of gelatine, inseparably casting on top of said separating layer a second silver halid layer of different color-sensitiveness casting a third silver halid layer of different color-sensitiveness on the other side of said base, producing the images by a single exposure, developing the partial images, treating the image layers to give the bottom layer its finish, hardening said operating layer, and treating the top layer to give it its finish.

6. A method of producing a color photograph comprising casting on a base a silver halid layer, forming on said layer a separating layer of gelatine, inseparably casting on top of said separating layer a second silver halid layer of different color-sensitiveness, producing the images by a single exposure, developing the partial images, dyeing the image layers, hardening said separating layer, and redyeing with a different colored dye the image layer on top of said hardened separating layer.

7. A method of producing a color photograph comprising casting on a base a silver halid layer, forming on said layer a separating layer of gelatine, inseparably casting on top of said separating layer a second silver halid layer of different color-sensitiveness, producing the images by a single exposure, developing the partial images, dyeing the images bluish red, hardening said separating layer, and treating with a bluish green dyestuff the image on top of said hardened separating layer to produce a pure blue color image.

FRIEDRICH LIERG.